# EUROPEAN PATENT APPLICATION

(11) **EP 0 511 018 A1**
(43) Date of publication of application: **28.10.1992**
(21) Application number: 92303745.1
(22) Date of filing: 24.04.1992
(51) Int. Cl.: G03G 5/05

(54) **Electrophotographic photoreceptor**

(30) Priority: 26.04.1991 JP 97301/91; 08.04.1992 JP 86938/92
(71) Applicant: MITSUBISHI KASEI CORPORATION, Tokyo 100 (JP)
(72) Inventor: Nozomi, Mamoru, Yokohama-shi, Kanagawa-ken (JP); Fuse, Masahiro, Machida-shi, Tokyo (JP)
(74) Representative: Woods, Geoffrey Corlett

(57) **Abstract**

An electrophotographic photoreceptor having on a conductive base a photoconductive layer comprising a charge generation material, a charge transport material, and an organic acid, whose acid dissociation constant pKa in aqueous solution is from 2.1 to 4.3, in an amount of from 0.001 to 10 parts by weight per 100 parts by weight of the charge transport material.

## Description

The present invention relates to an electrophotographic photoreceptor.

In recent years, electrophotography has been applied to copying machines as well as to various printers, because it can provide high quality images without delay. As a photoreceptor which plays an important role in electrophotography, a photoreceptor comprising an inorganic photoconductive substance such as selenium, an arsenic-selenium alloy, cadmium sulfide or zinc oxide has been used. More recently, a photoreceptor comprising an organic photoconductive substance was proposed. The latter has advantages, i.e. it is not a pollutant and it has film-formability and shapability.

As one of the organic photoreceptors, the so-called "laminated-type photoreceptor" in which a charge generation layer and a charge transport layer are successively laminated was developed. The laminated-type photoreceptor is increasingly of interest and is expected to be widely used in the near future because it has the following advantages:
(1) a photoreceptor having a high sensitivity can be obtained by suitably selecting and combining a charge generation material and a charge transport material;
(2) a photoreceptor having a high safety can be obtained because the charge generation material and the charge transport material can be selected from a wide range of the materials; and
(3) a photoreceptor can be prepared by a simple coating and thus can be prepared with low cost.

However, prior laminated-type photoreceptors have poor durability. When they are repeatedly used, electric problems such as a lowering in charged potential, an accumulation of residual potential and a change in sensitivity occur. The problem of accumulation of residual potential is especially serious because if residual potential is accumulated not many copies can be obtained. Such an accumulation of residual potential is considered to arise from various causes, among which impurities present in the charge transport layer are important. The impurities include impurities originally present in the composition used for forming the charge transport layer, impurities produced after the charge transport layer is subjected to a corona discharge and impurities produced by decomposition after the charge transport layer is exposed repeatedly during exposure steps and erasing steps and after the charge transport layer is subjected to outside light during maintenance. These impurities trap carriers and thus unmovable space charges which remain as residual charges in the charge transport layer are produced.

As another cause of lowering of the durability of the laminated-type photoreceptor, reduction in thickness of the charge transport layer due to mechanical stresses, for example by abrasion during blade cleaning, leading to lowering in electric properties, may also be mentioned.

An increase in the thickness of the charge transport layer is effective to prevent the reduction in thickness of the charge transport layer and increase the sensitivity of the photoreceptor, but it is accompanied with an increase in the amount of impurities, which increases accumulation of residual potential.

To prevent accumulation of residual potential caused by the impurities present in the charge transport layer, addition of a specific compound in the charge transport layer may be attempted. However, known compounds are not satisfactory because they insufficiently prevent accumulation of the residual potential and they affect the electric properties including the chargeability and sensitivity.

The present invention provides an electrophotographic photoreceptor having on a conductive base a photoconductive layer comprising a charge generation material, a charge transport material, and an organic acid, whose acid dissociation constant pKa in aqueous solution is from 2.1 to 4.3, in an amount of from 0.001 to 10 parts by weight per 100 parts by weight of the charge transport material.

The present invention also provides a copying machine or printer which comprises a photoreceptor as defined above.

The above organic acid can prevent the accumulation of residual potential sufficiently without affecting the electric properties.

The photoconductive layer may be a laminated-type photoconductive layer in which the charge transport layer and the charge generation layer are successively laminated, or a dispersion-type photoconductive layer in which the particulate charge generation material is dispersed in a medium containing the charge transport material and a binder resin.

As the conductive base, any known conductive base can be used. Examples are a base comprising a metal such as aluminium, stainless steel, copper or nickel as well as a base comprising an insulating material such as polyester film or paper on which a conductive layer such as a layer of aluminium, copper, palladium, tin oxide or indium oxide is provided.

The organic acid contained in the photoconductive layer in the photoreceptor of the invention should have the acid dissociation constant pKa in its aqueous solution in the range of 2.1 to 4.3. As the usable organic acid, aromatic carboxylic acids, saturated or unsaturated aliphatic carboxylic acids, sulfur-containing organic acids and phosphorus-containing organic acids, which may have any substituents such as halogen atom, and hydroxy, thiol, alkyl, aryl, nitro, amino, dialkylamino, alkoxy and aryloxy groups, are exemplified. Especially, the aromatic carboxylic acid which may be substituted as well as the saturated or unsaturated aliphatic carboxylic acid which may be substituted are preferable. Typical examples of the organic acids include acrylic acid, adipic acid, adenosine-2′-phosphate, valeric acid, 3-chloropropionic acid, acetic acid, cyanoacetic acid, phenylacetic acid, phenoxyacetic acid, bromoacetic acid, butyric acid, cyclohexanecarboxylic acid, o-anisic acid, 1-anilinesulfonic acid, p-aminobenzoic acid, benzoic acid, p-chlorobenzoic acid, m-hydroxybenzoic acid, o-nitrobenzoic acid, salicylic acid, 1-naphthoic acid, oxalacetic acid, succinic acid, tartaric acid, lactic acid, malic acid, phthalic acid, terephthalic acid, mandelic acid and crotonic acid.

In the laminated-type photoconductive layer, the organic acid can be contained in the charge generation layer and/or the charge transport layer. When it is contained in the charge generation layer, its amount is generally 0.001 to 10 parts by weight, preferably 0.01 to 2 parts by weight per 100 parts by weight of the charge transport material in the charge transport layer. On the other hand, when it is contained in the charge transport layer, its amount is generally 0.001 to 10 parts by weight, preferably 0.01 to 2 parts by weight per 100 parts by weight of the charge transport material in the charge transport layer. The inclusion of the organic acid in the charge transport layer is more preferable.

The charge generation layer in the laminated-type photoconductive layer contains the charge generation material. As the charge-generation material used in the charge generation layer or in the photoconductive layer, various inorganic photoconductive substances such as selenium or its alloys, arsenic-selenium alloy, cadmium sulfide and zinc oxide as well as various organic photoconductive substances such as phthalocyanine, azo pigment, quinacridone, polycyclic quinone, pyrylium salt, thiapyrylium salt, indigo, thioindigo, anthoanthrone, pyranthrone and cyanine can be used. Among them, the phthalocyanine without a metal; the phthalocyanine coordinated with the metal or its compound, for example coordinated with a metal oxide or a metal chloride, such as tin, zinc, vanadium, oxytitanium, tin chloride, copper indium chloride and gallium chloride; and the azo pigment such as monoazo, bisazo, trisazo and polyazo are preferable.

The charge generation material can be used in the charge generation layer together with at least one of binder resins such as polyester resin, polyvinyl acetate, polyacrylate, polymethacrylate, polycarbonate, polyvinyl acetacetal, polyvinyl propional, polyvinyl butyral, phenoxy resin, epoxy resin, urethane resin, cellulose ester and cellulose ether.

The charge generation material is preferably used in an amount of 30 to 500 parts by weight per 100 parts by weight of the binder resin.

If necessary, the charge generation layer may contain various additives such as a leveling agent, an antioxidant and a sensitizer.

The charge generation layer is usually formed on the conductive base according to any one of the known methods, preferably a coating method wherein a coating solution containing the charge generation material and the binder resin together with any optional additives in a suitable solvent is coated. Alternatively, the charge generation layer may be formed by directly depositing the charge generation material on the conductive base.

The thickness of the charge generation layer is generally 0.1 to 2 µm, preferably 0.15 to 0.8µm.

The charge transport layer contains the charge transport material and the binder resin. The charge transport material used in the charge transport layer or in the photoconductive layer is an electron donative material, the examples of which include heterocyclic compounds such as carbazole, indole, imidazole, oxazole, pyrazole, oxadiazole, pyrazoline and thiadiazole; aniline derivatives; hydrazone compounds; aromatic amine derivatives; stilbene derivatives and polymers having the above compound in their main chain or their side chain.

As the binder resin used together with the charge transport material in the charge transport layer, a vinyl polymer, for example a homopolymer or copolymer, such as polymethyl methacrylate, polystyrene and polyvinyl chloride and its copolymer, polycarbonate, polyester, polyester carbonate, polysulfone, polyimide, phenoxy resin, epoxy resin and silicone resin can be used. Their partially crosslinked products may be used.

The charge transport material is generally used in an amount of 30 to 200 parts by weight, preferably 40 to 150 parts by weight per 100 parts by weight of the binder resin.

If necessary, the charge transport layer may contain various additives such as the antioxidant and the sensitizer.

The charge transport layer is usually formed on the charge generation layer according to any of the known methods, preferably the coating method wherein the coating solution containing the charge transport material and the binder resin together with any optional additives in a suitable solvent is coated.

The thickness of the charge transport layer is generally 10 to 60 µm, preferably 10 to 45 µm.

The laminated-type photoconductive layer described in the above has the charge generation layer on which the charge transport layer is provided, but the order of laminating the charge generation layer and the charge transport layer may be changed, if necessary.

As an outer layer, a known overcoat layer, for example. a layer mainly composed of a thermoplastic or thermosetting polymer can be provided.

As mentioned in the above, the dispersion-type photoconductive layer comprises the particulate charge generation material dispersed in the medium containing the charge transport material and the binder resin. The ratio of the charge transport material to the binder resin is the same as that in the laminated-type photoconductive layer.

In the dispersion-type photoconductive layer, the charge generation material should have a small particle size. Its particle size is preferably 1 µm or less, more preferably 0.5 µm or less.

The charge generation material dispersed in the medium is preferably in an amount of 0.5 to 50 % by weight, more preferably in an amount of 1 to 20 % by weight based on the medium.

When the organic acid is contained in the dispersion-type photoconductive layer, its amount is generally 0.001 to 10 parts by weight, preferably 0.01 to 2 parts by weight per 100 parts by weight of the charge transport material in the photoconductive layer.

If necessary, the dispersion-type photoconductive layer may contain various additives such as a plasticizer, a dispersion assistant, a leveling agent and a surfactant.

The thickness of the dispersion-type photoconductive layer is generally 5 to 50 µm, preferably 10 to 45 µm.

### EFFECT OF THE INVENTION

The electrophotographic photoreceptor containing the specific organic acid in the photoconductive layer according to the invention shows very high sensitivity and low residual potential. It hardly shows the accumulation of the residual potential and the change in charge-ability and sensitivity, even if its repeated use. Therefore, it is excellent in the durability.

### EXAMPLES

The invention will be better understood by reference to certain examples, which are included herein for the purpose of illustration only and are not intended to limit the invention.

### Example 1

10 Parts by weight of a bisazo compound having the following formula:
were added to 150 parts by weight of 4-methoxy-4-methyl-pentanone-2 and they were subjected to the grinding and dispersion treatment using a sand grind mill. The thus obtained dispersion was added to 100 parts by weight of a 5 % solution of polyvinyl butyral (#6000-C (trade name), ex DENKI KAGAKU KOGYO K.K.) in 1,2-dimethoxyethane so as to prepare a dispersion with a solid concentration of 4.0 %.

The above dispersion was coated using a wire bar on a surface of a polyethylene terephthalate film having an aluminium deposited layer followed by drying, thereby the charge generation layer with a thickness of 0.4 g/m² was formed.

On the charge generation layer, a solution of 95 parts by weight of a hydrazone compound having the following formula:
1.5 parts by weight of 4-(2,2′-dicyanovinyl)phenyl 2,4,5-trichlorobenzene sulfonate, 0.2 part by weight of p-hydroxybenzoic acid (pKa 4.58) and 100 parts by weight of a polycarbonate resin having the following formula:
in a mixed solvent of 1,4-dioxane and tetrahydrofuran (volume ratio of 50:50) was coated using an applicator followed by drying at room temperature for 30 minutes and 125°C for 30 minutes, thereby the charge transport layer with a thickness of 35 µm was formed.

In this way, a laminated-type electrophotographic photoreceptor (sample A) was prepared.

### Examples 2 to 6

The procedures in Example 1 were repeated, except that p-hydroxybenzoic acid was replaced with other organic acids, o-nitrobenzoic acid of pKa 2.17 (Example 2, sample B), o-chlorobenzoic acid of pKa 2.92 (Example 3, sample C), 2-bromovaleric acid of pKa 2.7 (Example 4, sample D), 3-phenylsalicylic acid of pKa 2.8 (Example 5, sample E) and p-tert-butylbenzoic acid of pKa 4.2 (Example 6, sample F).

### Comparative Example 1

The procedure in Example 1 was repeated, except that p-hydroxybenzoic acid was omitted so as to prepare the photoreceptor (sample G).

### Comparative Example 2

The procedure in Example 1 was repeated, except that p-hydroxybenzoic acid was replaced with trichloroacetic acid (pKa 0.66) so as-to prepare the photoreceptor (sample H).

### Example 7

10 Parts by weight of a bisazo compound having the following formula:
and 0.2 part by weight of 2-bromovaleric acid (pKa 2.7) were added to 150 parts by weight of 4-methoxy-4-methyl-pentanone-2 and they were subjected to the grinding and dispersion treatment using a sand grind mill. The thus obtained dispersion was added to 100 parts by weight of a 5 % solution of polyvinyl butyral (#6000-C (trade name), ex DENKI KAGAKU KOGYO K.K.) in 1,2-dimethoxyethane so as to prepare a dispersion with a solid concentration of 4.0 %.

The above dispersion was coated on a surface of a polyethylene terephthalate film having an aluminium deposited layer using a wire bar followed by drying, thereby the charge generation layer with a thickness of 0.4 g/m² was formed.

On the charge generation layer, a solution of 95 parts by weight of a hydrazone compound having the following formula:
1.5 parts by weight of 4-(2,2′-dicyanovinyl)phenyl 2,4,5-trichlorobenzene sulfonate and 100 parts by weight of a polycarbonate resin having the following formula:
in a mixed solvent of 1,4-dioxane and tetrahydrofuran (volume ratio of 50:50) was coated using an applicator followed by drying at room temperature for 30 minutes and 125°C for 30 minutes, thereby the charge transport layer with a thickness of 35 µm was formed.

In this way, a laminated-type electrophotographic photoreceptor (sample I) was prepared.

### Example 8

The procedure in Example 7 was repeated, except that 2-bromovaleric acid was replaced with o-nitrobenzoic acid of pKa 2.17 so as to prepare the photoreceptor (sample J).

### Comparative Example 3

The procedure in Example 7 was repeated, except that 2-bromovaleric acid was omitted so as to prepare the photoreceptor (sample K).

### Test Example

The characteristics of the photoreceptors A to K prepared in Examples and Comparative Examples were tested.

Each photoreceptor was placed in an apparatus for determining the characteristics of the photoreceptor (Model EPA-8100, ex KAWAGUCHI DENKI K.K.) and charged so that the current flowing into the aluminium layer was 72 µA, followed by exposing and erasing. Then, the charge-ability (V₀), the dark decay (DD, the rate of decaying of the electrical potential in the dark after 2 seconds from the charging), the sensitivity of half decay exposure (E_{1/2}, reference potential 500 V) and the residual potential (Vᵣ) were determined.

The results are shown in Table 1

As clear from the results in Table 1, the electro-photographic photoreceptor according to the invention has the excellent properties.

### Example 9

The procedure in Example 1 was repeated, except that an aluminium cylinder having a diameter of 80 mm, a length of 340 mm and a thickness of 1 mm was used as the conductive base so as to prepare the cylindrical photoreceptor.

This photoreceptor was set in a commercial copying machine The images with high qualities could be obtained.

## Claims

1. An electrophotographic photoreceptor having on a conductive base a photoconductive layer comprising a charge generation material, a charge transport material, and an organic acid, whose acid dissociation constant pKa in aqueous solution is from 2.1 to 4.3, in an amount of from 0.001 to 10 parts by weight per 100 parts by weight of the charge transport material.

2. A photoreceptor according to claim 1 wherein the photoconductive layer is a laminated-type photoconductive layer comprising at least a charge generation layer and a charge transport layer.

3. A photoreceptor according to claim 2 wherein the organic acid is contained in both the charge transport layer and the charge generation layer.

4. A photoreceptor according to claim 1 wherein the photoconductive layer is a dispersion-type photoconductive layer wherein the charge generation material is dispersed in a medium containing the charge transport material and a binder resin.

5. A photoreceptor according to any one of the preceding claims wherein the organic acid is at least one selected from aromatic carboxylic acids which may be unsubstituted or substituted, saturated or unsaturated aliphatic carboxylic acids which may be unsubstituted or substituted, sulfur-containing organic acids which may be unsubstituted or substituted and phosphorus-containing organic acids which may be unsubstituted or substituted.

6. A photoreceptor according to claim 5 wherein the organic acid is an aromatic carboxylic acid which may be unsubstituted or substituted or an aliphatic carboxylic acid which may be unsubstituted or substituted.

7. A photoreceptor according to any one of the preceding claims wherein the organic acid is present in an amount of from 0.01 to 2 parts by weight per 100 parts by weight of the charge transport material.

8. A photoreceptor according to any one of the preceding claims wherein the conductive base comprises a metallic material or an insulating substrate having a conductive layer on its surface.

9. A photoreceptor according to any one of the preceding claims wherein the charge generation material is an organic photoconductive substance.

10. A photoreceptor according to any one of the preceding claims wherein the charge transport material is at least one electron donative material selected from heterocyclic compounds, aniline derivatives, hydrazone compounds, aromatic amine derivatives, stilbene derivatives and polymers having groups derived from any of the above compounds in their main chain or side chains.

11. A copying machine or printer which comprises a photoreceptor as defined in any one of the preceding claims.
